

June 14, 1938.

L. WILSON

2,120,319

METHOD OF ANNEALING

Filed June 15, 1935



*Fig. 1A.*



INVENTOR

Lee Wilson  
by his Attorneys  
Byrnes, Stabbins & Blenko

## UNITED STATES PATENT OFFICE

2,120,319

## METHOD OF ANNEALING

Lee Wilson, Cleveland, Ohio

Application June 15, 1935, Serial No. 26,853

1 Claim. (Cl. 148—21.5)

My invention relates to the art of treating metal and, in particular, to the annealing of thin gauge metal in strip form. The annealing of strip has always been attended with considerable difficulty heretofore. About the best procedure evolved so far is the annealing of strip in coils in which it is reeled after cold rolling, either in conventional annealing boxes or in boxes particularly designed to receive round coils. The boxes may be heated by heating means mounted therein, or may be bodily movable into a heating furnace. In either case, the annealing process is very slow and the efficiency is not very high, particularly as to the stacking of coils in conventional annealing boxes. A large amount of equipment is necessary because of the slowness of the process, and this makes the operation very expensive.

My invention overcomes the aforementioned objections to the present practice of annealing strip and provides, for the first time, so far as I am aware, a practical, inexpensive and rapid method of annealing strip. In accordance with my invention, I anneal strip by heating it to the required temperature while in strand form. I coil the strip while still hot and cool it slowly in the coiled form. The heating, coiling and cooling operations are preferably conducted in the absence of atmospheric oxygen. I stitch together successive strips being annealed and sever the strip when a sufficient amount thereof has been coiled from the strand. I also prefer to cool the strip slightly before coiling to prevent sticking of successive turns of the coil and for metallurgical reasons. My invention also includes a novel form of coiling apparatus particularly adapted for the performance of the method outlined above, and an annealing furnace of novel construction.

A present preferred embodiment of the apparatus for carrying out the invention is illustrated in the accompanying drawing and will be described particularly in connection with the following explanation of the method. In the drawing,

Figure 1 is a longitudinal vertical section through an annealing furnace and a portable coiling device, in accordance with my invention;

Figure 1A is a similar view of the coiling device and a cooling chamber; and

Figure 2 is a sectional view taken along the line II—II of Figure 1.

Referring now in detail to the drawing, an annealing furnace 10 of the so-called "tunnel" type, has side walls 11, a roof 12 and a hearth 13 com-

posed of refractory material assembled within a structural framework (not shown). The entrance end of the furnace has a restricted port or opening 14 normally closed by flexible flaps 15 which are displaceable by strip material indicated at 16 moving into the furnace. The discharge end of the furnace is provided with an opening or port 17.

The interior of the furnace is divided by a transverse partition wall 18 into a heating chamber 19 and a cooling chamber 20. Pinch roll stands 21 and 22 located at the entrance end of the furnace and adjacent the discharge opening 17, respectively, serve to feed the strip through the furnace in the direction of the arrow 23. Conveyor rollers 24 are mounted at intervals along the length of the furnace to support the material being passed therethrough.

The heating chamber 19 is provided with a plurality of heat exchange tubes 25. In the particular form of the invention illustrated, the tubes extend transversely of the furnace chamber and penetrate the side walls 11 thereof at points above the rolls 24. Any other suitable arrangement of the tubes may, however, be employed. Burners 26 extend into the tubes adjacent one end, the other end of each tube being open for discharging combustion gases. A damper 27 is mounted adjacent the discharge end of each tube for controlling the flow of gases therethrough. Fuel is supplied to the burners 26 from headers 28 and air for combustion is induced through the open ends of the tubes in which the burners are mounted.

The cooling chamber 20 is also provided with conveyor rolls 24. Heat exchange tubes 20a extend transversely of the furnace above the conveyor rolls and are connected to any suitable source of cooling medium, such as air. The function of the tubes 20a is to cool the material 16 slightly before it emerges from the furnace.

A portable coiler 30 comprises a frame 30 preferably provided with wheels 31 for easy movement, and an enclosure 32 of any suitable construction. A coiler 33 is mounted on the frame 30 within the enclosure 32. The construction of coilers is well known and requires no detailed disclosure.

At one side, the enclosure 32 is provided with a tubular projection 34 adapted to enter the port 17 and make a substantially gas-tight connection therewith. The enclosure 32 is also provided with a door 35 which may be hinged or slidably mounted for opening.

A cooling chamber 36 of any suitable construc-

tion and preferably having a door 37, is disposed in any desired location, preferably adjacent the furnace 10. The function of the cooling chamber is to receive coils of strip for slow cooling after they have been heated to the annealing temperature and, so long as it performs its function, the specific construction thereof is not of great moment.

The method of my invention will now be explained referring to the apparatus already described. Strip metal is usually rolled in relatively long lengths and coiled when the rolling is completed. It may be assumed, therefore, that the material 16 entering the furnace 10 is unwound from a coil mounted on an uncoiler. Alternatively, the strip may be fed directly from the mill to the furnace. The first length of strip may be fed through the furnace by means of a rigid leader in a manner well known to the art, and successive lengths of strip may be attached by spot welding or otherwise, to the trailing end of the preceding length, so as to form a continuous movement of successive strips through the furnace. The heating chamber of the furnace is preferably maintained at a temperature of 1500° F. to 1800° F. The strip is heated to this temperature gradually as it passes through the furnace, and the length of the furnace and the rate of travel of the material therethrough may be coordinated to insure the desired heating of the strip. As the strip enters the cooling chamber 20, it is cooled rapidly to about 1250° F. or any other desired temperature. I preferably maintain a non-oxidizing atmosphere within the chambers 19 and 20 of the furnace to prevent oxidation of the strip by atmospheric oxygen. This deoxidizing atmosphere also fills the enclosure 32 of the coiler 29 by virtue of the connection 34 between the enclosure and the cooling chamber 20. The strip on emerging from the furnace passes through the tubular connection 34 and on to the coiler 33. The strip is thus coiled at a temperature of substantially 1250° F., in a non-oxidizing atmosphere. When a sufficient amount of strip has been coiled, the coiler 29 is pulled away from the furnace and the strip severed adjacent the port 17. The coiler is then moved to the cooling chamber 36, the door 37 of which is opened, to permit the coil formed by the coiler 33 to be removed therefrom through the door 35 and deposited in the cooling chamber. If desired, the open end of the tubular projection 34 may be temporarily closed by any suitable cover while the coiler is being removed to the cooling chamber 36. When the hot coil has been placed in the cooling chamber, the coiler is re-

turned to the position shown in Figure 1 and a new coil is started.

After a period of slow cooling in the chamber 36, the annealing is completed and the coils may be removed therefrom for further manufacturing operations.

The rapid cooling step of the process is not necessary when annealing certain material, such as silicon steel or corrosion-resistant steel alloys, because such materials are not subject to sticking of adjacent turns of the coil at the normalizing temperature above mentioned, viz., around 1500 to 1800° F.

It will be apparent that the invention described in the foregoing constitutes a marked improvement over present processes of annealing. The rate of performing the annealing operation is greatly increased and only a relatively small amount of equipment is necessary. Since the material passes through the furnace rather rapidly, the tonnage output is high. The chamber in which the coils are slowly cooled may be of relatively inexpensive construction and easily designed for almost any desired capacity. The invention also lends itself admirably to bright annealing, since all the operations can be conducted in the absence of atmospheric oxygen.

The portable coiler makes it possible to conduct the cooling operation in a non-oxidizing atmosphere and thereby protect the strip being coiled from atmospheric oxidation. The coiler also serves as a convenient means for transporting coils from the furnace to the cooling chamber.

The indirect heating of the annealing furnace is advantageous in that it insures a substantially uniform temperature throughout the furnace and prevents overheating of or injury to the material being treated, which might result from direct contact of the hot combustion gases therewith.

Although I have illustrated and described herein but one preferred form and practice of the invention, it will be apparent that any changes in the apparatus and method disclosed may be made without departing from the spirit of the invention or the scope of the appended claim.

I claim:

A method of annealing a steel strip including the steps of heating the strip in strand form to a temperature of about 1300° F. or above, cooling the strip rapidly to a lesser elevated temperature but sufficiently below 1300° F. to prevent sticking of turns when coiled, coiling the strip at said temperature, and thereafter cooling the coiled strip slowly to room temperature.

LEE WILSON.

55